

## UNITED STATES PATENT OFFICE

2,635,958

## METHOD OF PRODUCING POROUS PAPER

Daniel S. Dieffenderfer, Easton, Pa., and Andrew Loy Moore Bixler, Milford, N. J., assignors to Riegel Paper Corporation, New York, N. Y., a corporation of New Jersey

No Drawing. Original application February 4, 1947, Serial No. 726,446. Divided and this application April 14, 1949, Serial No. 87,564

3 Claims. (Cl. 92—21)

1

This invention relates to improvements in the method of producing porous paper.

More particularly the invention relates to a method of producing a strong, highly porous paper having special properties which make it valuable for use for filtering air as in vacuum cleaner bags.

According to the present invention, admixed leather fibers and cellulose fibers in suitable proportions are formed into a wet sheet and the wet sheet is subjected to a heating treatment while still wet to effect shrinkage, decomposition and change in the leather fibers to produce a special porous sheet of paper containing the cellulose fibers bound together by the modified leather particles.

Particularly advantageous porous paper can be made from admixtures of leather fibers and long cellulose fibers in approximately equal proportions, but these proportions can be somewhat varied, for example, between 40 and 60% leather fibers and between 60 and 40% of long cellulose fibers for the production of highly porous paper adapted for filtering air. A somewhat lower proportion of leather fibers, down to around 20%, and a somewhat higher proportion, up to around 70%, can be used to give paper of modified properties which is less valuable for air filtering purposes but adapted for other purposes.

The leather fibers used in making the new paper may be ordinary leather fibers obtained by shredding or fiberizing leather waste or scrap which is shredded or divided so that the fibers are separated more or less completely and present a fibrous structure and appearance adapting them for use in paper manufacture. The cellulose fibers may be of any type that can be formed into a web on a paper machine. For the purpose of the product herein described, long, strong cellulose fibers are best adapted. Since the leather fibers are dark in color and darken even more during shrinkage and decomposition, unbleached fibers are well adapted. Among such types which are found very suitable are strong krafts, rope and jute.

The admixture of leather and cellulose fibers and the production of an admixed pulp therefrom can be carried out in ordinary pulp making equipment. Thus the pulp may be prepared by the following procedure.

The cellulose fibers such as unbleached Kraft pulp are supplied to the beater first and are beaten to the desired freeness, advantageously in the range of 700 cc. to 500 cc. as measured by a Canadian freeness tester. The exact freeness selected for a particular application depends on the porosity and strength properties desired in

the final sheet. In this particular case, we have found a freeness below 500 cc. to be undesirable. The leather fibers are next added to the beater, using e. g., tanned scrap leather in a fibrous form. Different percentages of leather, based on the total dry weight, will give varying amounts of porosity and dry and wet strength in the final sheet. For the production of vacuum cleaner bag paper a mixture of approximately 50% leather fibers and 50% cellulose fibers has been found to give the desired high porosity and sufficient overall strength. After the addition of the leather fibers to the beater, the mixture is run in the beater only long enough to thoroughly wet the leather fibers, to distribute them evenly through the furnish and reduce the stock to a slowness that will give the desired properties in the final sheet. The resulting freeness of the furnish is in the range of about 500 cc. to 200 cc. depending on the freeness of the material first furnished in the beater and the length of time the combined furnish is run. The stock is now ready for the paper machine.

The pH of the stock should not be changed to any great extent from the normal resulting pH produced by the leather fibers, other fibers and water in the beater. This normal pH is in the range of around 4.5 in the beater to 6.5 in the headbox. A lowering of the pH below about 4.0 tends to retard the shrinkage and decomposition of the leather during the subsequent heating on the steam dryers with resulting lowering in porosity, while too high a pH, around 8.0 or higher, tends to cause the leather to decompose or dissolve in the stock mixer, thus tending to lose the effect of the shrinkage and decomposition which is desired on the steam dryers.

The prepared furnish from the beater is supplied to an ordinary paper making machine and a wet sheet of paper is produced. The drying of this sheet in the ordinary way on a paper machine does not produce the new porous paper. To produce the desired porous paper it is important to subject the wet sheet to a high temperature while the leather fibers are still wet.

It appears that the wet leather fibers on being heated to a sufficiently high temperature tend to soften and swell and to decompose, becoming somewhat gelatinous so that they adhere to the adjacent cellulose fibers. In order to produce the new porous paper extreme shrinkage of the leather fibers and more or less decomposition on heating of the wet fibers appears necessary. The gelatinized leather fibers appear to glue the cellulose fibers together. The leather remains in this relatively swollen gelatinized condition until the initial shrinking temperature is reached, around

160° F., when a marked shrinkage and more or less decomposition of the leather fibers takes place. This shrinkage is of such a degree that irregular voids are created in the sheet, not only by the loss of volume of the leather fibers, but by the effect of the leather in distorting the cellulose fibers to which it is adhered. The leather remains gummy and sticky during the shrinking and appears to remain tacky and gummy until it becomes quite dry.

As opposed to ordinary paper making practice, in which the first dryers are running at a lower temperature with gradual increase up to a higher temperature in the last dryers, the heating of the wet sheet containing the leather fibers is effected by using a high temperature on the first dryers so that the necessary heating to a high temperature and swelling and decomposition will take place before the sheet is dried. The temperature of the first dryers in the drying system over which the wet composite paper sheet is passed should have a surface temperature of around 250° F. or higher.

When such a high temperature dryer is used the composite wet sheet is rapidly heated to a temperature, e. g., around 160° F. or somewhat higher so that prior to the actual drying and removal of water the leather fibers are caused to soften and swell and become gelatinous and adherent to the cellulose fibers. The fiber structure of the leather is largely though not completely lost during this heating and drying operation. Some of the leather material apparently forms an adhesive solution and there is probably some complete thermal decomposition. The leather remaining is distributed through the sheet as a mixture of hard, amorphous particles and fibers; but because of the cellulose fibers the sheet as a whole retains sufficient flexibility and strength. The dried sheet is very porous and has a rough surface due to the changes that take place in the leather during the high temperature heating and drying.

One of the important properties imparted to the sheet by the gelatinized, shrunk and dried leather is that the leather cements the cellulose fibers together with a bond that retains a considerable proportion of its dry strength when the resulting paper is wet. This imparts to the sheet what is commonly called in papermakers' language wet strength. In ordinary paper made of cellulose fibers the bond strength between cellulose fibers is reduced to practically nothing when a sheet becomes wet and a sheet is said to lack wet strength. But the action of the modified leather fibers, according to the present invention, gives a paper having wet strength which makes the paper desirable for use under conditions where it may become wet during use. The improved highly porous sheet of paper produced by the present invention combines this high porosity with a wet strength comparable to or superior to that obtained with the ordinary wet strength agents used in the paper making industry.

The porosity of the paper sheet resulting from carrying out the invention has characteristic and distinctive properties. The shrinking of the swollen, gelatinized leather fibers on heating to effect partial decomposition causes shrinkage to such a degree that irregular voids are created in the sheet. These voids are created not only by the loss in volume of the leather fibers but by distortion of the cellulose fibers caused by the gummy and sticky leather fibers as they shrink and partially decompose. The resulting dried

sheet has a characteristic rough surface due to the changes in the sheet which take place in the leather fibers as they swell and shrink while adhering to the cellulose fibers. The sheet surface becomes hard and dry during the heating and drying operation, with an irregular broken surface. The sheet is not only very porous but microscopic examination indicates that the pores in the sheet are of varying size.

10 The present invention is particularly valuable for producing paper for use in filtering air, for example, for use in making vacuum cleaner bags, where it is important to filter dust and dirt from the air and permit the air to pass through. The variation in pore size in the sheet, together with the rough surface, greatly retards the increase in resistance to air flow as solid material (dust) is filtered out of the air on the surface, preventing the dust from collecting in a continuous, impervious film.

20 In contrast with porous sheets of paper made entirely of cellulose fibers with low initial resistance to air flow, where the resistance increases rapidly as solid particles collect on the surface, which is relatively plain, and form a continuous relatively impervious film of dust which quickly forms and plugs the paper and interferes with its filtering action, the improved 25 porous paper made in accordance with the present invention, with its rough, uneven surface and is characteristic interior porosity, permits effective filtering of solid material (dust) for prolonged periods of time without the formation of a continuous, impervious film.

30 The new paper sheet produced by the present method can be somewhat further improved in wet strength by treating the sheet after it is formed with added wet strength agents. Such agents should not in general be added at the beater or headbox since the acid condition required in such cases interferes with the conversion of the leather on subsequent heating and tends to reduce porosity. But by applying an added wet strength agent by a size press application after the composite sheet has been formed and dried, somewhat increased wet strength can be imparted to the sheet without the loss of the desirable high porosity of the sheet.

35 The important characteristics of composite paper made in accordance with the new method 40 will be illustrated by tests carried out on sheets made with varying proportions of leather and cellulose in the furnish which has been formed into a sheet and heated to bring about the shrinkage and decomposition of the leather fibers by 45 heating the wet sheet to an elevated temperature at an early stage of the drying operation.

50 Sheets of paper were made from leather fibers and kraft fibers in the proportions indicated in the following table and tests were made for 55 porosity, the time shown in the table being for porosity for four sheets, 400 cc. drop as measured with the Gurley Densometer. The sheet weight was 50/500 from a furnish of 300 cc. free-ness. The following results were obtained:

|    | Furnish                     | Porosity 4 sheets/400 cc. |
|----|-----------------------------|---------------------------|
|    |                             | Sec.                      |
| 70 | 0% leather, 100% kraft..... | 88.                       |
|    | 10% leather, 90% kraft..... | 42.                       |
|    | 20% leather, 80% kraft..... | 42.                       |
|    | 30% leather, 70% kraft..... | 38.                       |
|    | 40% leather, 60% kraft..... | 16.                       |
|    | 50% leather, 50% kraft..... | 1.                        |
|    | 60% leather, 40% kraft..... | less than 1.              |

A further series of tests were carried out to show the effect of freeness on porosity of a sheet made of 50% leather and 50% kraft fibers, with the following results:

| Freeness, cc. | Porosity 4<br>sheets/400 cc. |
|---------------|------------------------------|
| Sec.          |                              |
| 550           | less than 1.                 |
| 400           | Do.                          |
| 350           | 1.                           |
| 300           | 1.                           |

The improved wet strength imparted to the sheet is illustrated by the following table, the sheets being those above described made from varying percentages of leather fibers and kraft fibers and the wet strength being indicated as % retention of Mullen strength by the wet sheet with the varying percentages of leather fibers in the furnish:

| Furnish                | Percent<br>Retention<br>of Mullen |
|------------------------|-----------------------------------|
| 0% leather, 100% kraft | 0                                 |
| 10% leather, 90% kraft | 5                                 |
| 20% leather, 80% kraft | 11                                |
| 30% leather, 70% kraft | 20                                |
| 40% leather, 60% kraft | 25                                |
| 50% leather, 50% kraft | 30                                |
| 60% leather, 40% kraft | 35                                |
| 70% leather, 30% kraft | 50                                |

The further improvement resulting from the treatment of the finished sheet by the addition of wet strength agents, applied in the size press to a sheet made of 50% leather and 50% kraft fibers with a furnish of 350 cc. freeness is indicated by the following table:

| Wet Strength Agent                     | Percent<br>Retention<br>of Mullen |
|----------------------------------------|-----------------------------------|
| None                                   | 33                                |
| 2% Glyoxal                             | 58                                |
| 3% Urea formaldehyde resin (U. F. 470) | 67                                |

From these tests it will be evident that a very marked increase in porosity is obtained even with 10 to 30% leather fibers admixed with the kraft fibers, while a particularly porous sheet is obtained with around equal proportions of leather and kraft fibers. It will also be seen that the new method produces a sheet of paper which retains a marked wet strength which can be somewhat further improved by further treatment of the finished sheet with other wet strength agents.

It will thus be seen that the present invention provides an improved sheet of paper characterized by high and distinctive porosity, having a hard, rough surface and containing long cellulose fibers bonded together and spaced apart by the modified leather fibers which are caused to pass through a swelling and gelatinizing and decomposing and shrinking treatment to give irregular shrunk particles and fibers of leather in the final product which bind the cellulose fibers together and also hold them spaced apart to give a characteristic, irregular porosity to the sheet.

It will further be seen that the composite sheet made in accordance with the present method, particularly when about equal proportions of leather and cellulose fibers are used, forms a

valuable filter paper for filtering air and for use in vacuum cleaner bags to replace the ordinary cloth bags, commonly used for that purpose.

It will also be seen that the invention provides an improved porous sheet which combines high porosity with sufficient strength and that the sheet retains its strength to a very large extent when wet, thus being adapted to use under conditions where the paper may become wet in use. And it will further be seen that still further improved wet strength can be imparted by the subsequent treatment of the paper, after the completion of its formation, by other wet strength agents.

The present invention provides an improved method which can be carried out in ordinary paper making apparatus and by ordinary paper making procedures, except for the important change in procedure involved in heating the wet sheet to a high temperature to effect swelling and gelatinizing and shrinkage and partial decomposition of the leather fibers. This important modification of the present paper making operation is however readily carried out by using high temperature in the first drying cylinders on which the wet paper is passed, with heating of the cylinders to temperatures around 250° F. or higher and with heating of the interior of the sheet to temperatures around 160° F. or somewhat higher. This rapid and immediate heating of the wet sheet prevents the drying of the leather fibers at low temperature and insures that the leather fibers are subjected to the necessary high temperature while still wet to cause them to adhere to the cellulose fibers and to shrink into irregularly shaped particles which serve as binding and spacing particles for binding the cellulose fibers together while holding them in spaced condition to give a characteristic and distinctive and desirable interior porosity and a characteristic porous and rough surface.

This application is a division of our application Serial No. 726,446, filed February 4, 1947, now abandoned.

45 We claim:

1. The process of producing paper of high porosity and wet strength which consists of admixing leather fibers and long cellulose fibers in proportions such that the leather fibers make up from about 20% to 70% of the mixture, forming a wet sheet from a pulp of such admixed fibers, rapidly heating the resulting wet sheet and the leather fibers contained therein to a high temperature of at least around 160° F. but insufficient to char the fibers while said leather fibers are still wet, to cause adhesion of the leather fibers to the cellulose fibers and shrinking and partial decomposition and gelatinizing of the leather fibers, said rapid heating of the wet sheet being effected by passing the sheet first over drying rolls heated to a surface temperature of at least about 250° C. and subsequently drying the resulting sheet.

2. The process according to claim 1, in which the leather fibers comprise from about 40% to 60% of the mixture.

3. The process according to claim 1 in which approximately equal proportions of leather fibers and long cellulose fibers are used.

DANIEL S. DIEFFENDERFER.  
ANDREW LOY MOORE BIXLER.

(References on following page)

## References Cited in the file of this patent

## UNITED STATES PATENTS

| Number    | Name         | Date          | 5  |
|-----------|--------------|---------------|----|
| 1,857,497 | Clapp        | May 10, 1932  |    |
| 2,011,914 | Schwartz     | Aug. 20, 1935 |    |
| 2,016,447 | Katze-Miller | Oct. 8, 1935  |    |
| 2,036,466 | Ellis        | Apr. 7, 1936  |    |
| 2,104,996 | Ives         | Jan. 11, 1938 | 10 |
| 2,140,189 | Mason        | Dec. 13, 1938 |    |
| 2,220,047 | Mason        | Oct. 29, 1940 |    |
| 2,237,235 | Lynam        | Apr. 1, 1941  |    |

## FOREIGN PATENTS

| Number  | Country       | Date          |
|---------|---------------|---------------|
| 154     | Great Britain | of 1856       |
| 1,278   | Great Britain | of 1856       |
| 2,720   | Great Britain | of 1870       |
| 522,880 | Great Britain | June 28, 1940 |

## OTHER REFERENCES

Manufacture of Pulp & Paper, 3d. ed., vol. V.,  
sec. 1, pp. 199, 203 (1939), pub. by McGraw-Hill,  
New York.